

## UNITED STATES PATENT OFFICE

2,003,960

## PRINTING

Ronald Tonkin and James Stevenson Wilson,  
Earl's Road, Grangemouth, Scotland, assignors  
to Imperial Chemical Industries Limited, a  
corporation of Great Britain

No Drawing. Application June 8, 1932, Serial  
No. 616,098. In Great Britain June 16, 1931

20 Claims. (Cl. 8—6)

This invention relates to new and improved printing pastes and color printing, and more particularly to the production and use of new printing pastes for vat colors.

5 In the process of textile printing, in which the textile material is first printed with a thickened paste of the color with substances such as gum and starches, with or without added alkalies and reducing agents and assistants, and then aged 10 by passing through a steaming chamber, improper and uneven fixation of the color present in the printing paste is liable to be encountered.

15 It is an object of the present invention to avoid or reduce the foregoing disadvantages. Further objects are the provision of new printing assistants, new printing pastes, and a new and improved process of printing. A still further object is the production and use of highly efficient 20 vat color printing pastes. Other objects will appear hereinafter.

These objects are accomplished according to 25 this invention by incorporating or including with printing pastes quaternary base compounds of the following general formula:



30 where  $R_1$ ,  $R_2$ ,  $R_3$  and  $R_4$  represent the same or different alkyl or aralkyl groups, one at least of which contains a hydroxy radical, and where  $X$  represents  $-\text{OH}$  or the residue of an acid. These 35 new printing assistants may be employed alone or in conjunction with other printing assistants.

The invention will be further illustrated but is not limited by the following examples, in which the parts are by weight.

40

## Example I

A printing paste is prepared according to the following recipe:

|                                             | Parts |
|---------------------------------------------|-------|
| 3:3'-dichloro-dianthraquinone 1:2:2':1'-di- |       |
| hydroazine, single strength paste           | 5     |
| British gum thickening                      | 9     |
| Glycerine                                   | 2     |
| Rongalite C                                 | 1.8   |
| Potash                                      | 3.2   |
| Choline chloride                            | 2     |

25

55 Cotton cloth is printed with the foregoing paste in the usual way, that is, by passing the cloth to be printed under some tension and pressure over an intaglio metal roll, the engraving of 60 which is filled with the printing paste. After

leaving the printing machine the printed cloth is passed into a drier whereby the printing paste is dried on the cloth in its proper place and the dye is prevented from spreading to other portions of the fabric. In order to complete the 5 printing, the cloth, after leaving the drier, is passed into a steam ager for a period of a few minutes during which time the vat color undergoes reduction and passes to the fiber. The fabric is then subjected to oxidizing conditions 10 which may include passing it into a steeping bath, usually of water or water containing an oxidizing agent. Any excess color is washed off in a soap solution with which the textile material is treated following the steeping. The printed material possesses stronger and brighter 15 shades than are obtained without choline chloride.

## Example II

5

Instead of the dye 3:3'-dichloro-dianthraquinone-1:2:2':1'-dihydroazine, Caledon brown RS (4:5'-di(benzoylamino)-1:1'-dianthraquinonyl carbazole) paste is used in the printing paste of Example I with good results.

25

## Example III

20

A printing paste is prepared according to the following recipe:

|                                             | Parts |
|---------------------------------------------|-------|
| 3:3'-dichloro-dianthraquinone 1:2:2':1'-di- |       |
| hydroazine, single strength paste           | 5     |
| British gum thickening                      | 11    |
| Glycerine                                   | 2     |
| Rongalite C                                 | 1.8   |
| Potash                                      | 3.2   |
| Choline chloride                            | 2     |

25

40 Cotton cloth is printed with this paste, dried, and steamed in the ager. The printed material possesses stronger and brighter shades than are obtained without choline chloride.

45

## Example IV

4:4'-dimethyl-6:6'-dichlorothioindigo paste with 50 very desirable results.

The new printing assistants preferably employed in accordance with the invention are quaternary base compounds as already defined which are non-volatile or substantially non-volatile under the conditions of operation and which are strong bases or salts of strong bases and which are hygroscopic or deliquescent. The results obtained with choline chloride in particular have 55 60

been very highly advantageous. This compound may be represented by the following formula:



As further examples of the new printing assistants falling within the invention may be mentioned compounds having the following formulæ:



75 as already defined). Quaternary base compounds containing other stable acid residues such

as, for example, phosphates may be classified similarly.

In practicing the invention, especially desirable results have been obtained in printing vat colors of the indanthrone series, particularly 3:3'-dichloro - dianthraquinone-1:2:1':2'-dihydroazine. As examples of other printing colors may be mentioned: Caledon blue RC, 6:6' diethoxy thioindigo, 7:7' dimethyl 5:5' dichlorothioindigo, 10 5:6:5':6' tetrabromindigo, bis- beta naphthio- 10 naphthene indigo and 4:4' dichlor-5:5' dibromindigo.

As is well known a composition of printing paste may vary widely with different dyes and manufacturers but, in the case of vat colors, 15 usually consists of a mixture of an unreduced vat dye, a strong reducing agent such as, sodium hydrosulphite or Rongalite, an alkali and a thickening agent. The thickening agent is usually a gum (for instance British gum), starch or both. Printing paste is usually prepared by mixing a dye paste or pastes with the other ingredients enumerated, said other ingredients being in the form of a gummy mixture generally called a printing gum. The dye pastes are 20 essentially finely divided suspensions of the dye with or without a dispersing agent. Printing assistants may be added to the dye paste or to the printing gum or the printing paste as desired. 25

The amount of printing assistant may vary 30 within relatively wide limits but may ordinarily be varied directly with the amount of dye. Empirical tests can usually be made to determine the optimum amount of printing assistant for any given dye. Very satisfactory results are obtained with proportions of printing assistant described in the examples but greater or lesser amounts may be employed if desired. 35

The process of the invention gives particularly 40 valuable results with regard to fullness and brightness of shade when the sub-stratum upon which the color is printed is mercerized cotton. Good results are also obtained in printing other cotton materials and, in general, materials which may be printed with vat colors including viscose rayon 45 and other fibers, fabrics and yarns of vegetable origin.

While the invention is not limited to any theory, inasmuch as the quaternary bases employed as printing assistants are, in general, very 50 deliquescent substances it appears probable that this property of deliquescence is partly or wholly responsible for the improved results which are obtained by their use. It may be that their presence assists in the absorption of water either before or during the steaming operation, by which means the conditions requisite for the proper fixation of the color are attained. They may also, in some cases, exert a solvent action on the color. 55

Most deliquescent inorganic salts are incompatible with the alkaline mixtures used in printing, especially with vat colors, being decomposed to give difficultly soluble hydroxides, oxides or carbonates with a reduction of the amount of alkali present in the printing paste due to the 60 formation of alkali salts; calcium chloride and ammonium nitrate may be taken as examples of such inorganic salts.

As previously indicated, the invention is particularly advantageous in that the presence of 70 these assistants in the printing paste makes possible the production of prints of superior strength and brightness to those obtained from a similar printing paste from which the assistant has been omitted. Moreover, the efficiency of these assist- 75

ants is such that by their use greatly improved prints may be obtained with dyes which are ordinarily poor printing colors such as, for example, 3:3'-dichloro-dianthraquinone-1:2:2':1-dihydroazine.

As many apparent and widely different embodiments of this invention may be made without departing from the spirit thereof, it is to be understood that we do not limit ourselves to the foregoing examples or description except as indicated in the following claims.

We claim:

1. Vat dye pastes comprising a water-insoluble vat dye and a quaternary base compound of the general formula



20 where  $R_1$ ,  $R_2$ ,  $R_3$  and  $R_4$  are the same or different alkyl or aralkyl groups, one at least of which is an alkyl group containing a hydroxy group, and where  $X$  represents  $-\text{OH}$  or an acid residue.

25 2. Vat dye textile printing pastes comprising a water-insoluble vat dye and choline or a salt thereof.

3. Vat dye printing pastes comprising a water-insoluble vat dye and a water-soluble quaternary base compound of the general formula



35 where  $R_1$ ,  $R_2$ ,  $R_3$  and  $R_4$  are the same or different alkyl groups, one at least of which contains a hydroxy group, and where  $X$  represents  $-\text{OH}$  or an acid residue.

40 4. Vat dye printing pastes comprising a water-insoluble vat dye and a water-soluble quaternary base compound of the general formula



45 where  $R_1$ ,  $R_2$ ,  $R_3$  and  $R_4$  are the same or different alkyl or aralkyl groups, one at least of which is an alkyl group containing a hydroxy group, and where  $X$  represents an inorganic acid residue.

50 5. A vat dye paste comprising a water-insoluble vat dye and choline chloride.

6. Printing pastes comprising an anthraquinone vat dye and a water-soluble quaternary base compound of the general formula



55 60 where  $R_1$ ,  $R_2$ ,  $R_3$  and  $R_4$  are the same or different alkyl or aralkyl groups, one at least of which is an alkyl group containing a hydroxy group and where  $X$  represents  $-\text{OH}$  or an acid residue.

7. A process of printing textiles comprising adding to a paste containing a vat dye and other customary ingredients a water-soluble quaternary base compound of the general formula



70 where  $R_1$ ,  $R_2$ ,  $R_3$ , and  $R_4$  are the same or different alkyl or aralkyl groups, one at least of which is an alkyl group containing a hydroxy group and where  $X$  represents  $-\text{OH}$  or an acid residue and

thereafter using the compounded paste in printing.

8. A process of printing textiles as claimed in claim 7 wherein the paste contains a vat dye and choline or a salt thereof.

9. A process of printing textiles as claimed in claim 7 wherein the dyestuff is 3:3'-dichloro-dianthraquinone-1:2:2':1'-dihydroazine.

10. A process of printing textiles as claimed in claim 7 wherein the dye is a chloro dianthraquinone-1:2:2':1'-dihydroazine.

11. A process of printing textiles as claimed in claim 7 wherein the paste contains a chloro dianthraquinone-1:2:2':1'-dihydroazine and choline chloride.

12. A dye paste of a halogenated dianthraquinone-1:2:2':1'-dihydroazine containing as an ingredient choline chloride.

13. A dye paste of a chloro dianthraquinone-1:2:2':1'-dihydroazine containing as an ingredient choline chloride.

14. A dye paste of 3:3'-dichloro-dianthraquinone-1:2:2':1'-dihydroazine containing as an ingredient choline chloride.

15. A thioindigoid dye paste containing as an ingredient choline chloride.

16. A dye paste of 4:4'-dimethyl-6:6'-dichlorothiindigo containing as an ingredient choline chloride.

17. A dye paste of a di(benzoylamino)-1:1'-dianthraquinonyl carbazole containing as an ingredient choline chloride.

18. A dye paste comprising a water insoluble vat dye and a water-soluble quaternary base compound of the general formula:



wherein  $R_1$ ,  $R_2$ ,  $R_3$  and  $R_4$  are the same or different alkyl groups not containing more than two carbon atoms, one at least of which is a hydroxy ethyl group, and where  $X$  represents  $-\text{OH}$  or an inorganic acid residue.

19. A printing paste comprising a vat dye, an alkali, a reducing agent suitable for printing, a gum thickening agent, and a quaternary base compound of the general formula:



wherein  $R_1$ ,  $R_2$ ,  $R_3$  and  $R_4$  are the same or different alkyl or aralkyl groups, one at least of which is an alkyl group containing a hydroxy group, and where  $X$  represents  $-\text{OH}$  or an acid residue.

20. The process of printing vat dyes which comprises applying to the fiber a printing paste comprising the vat dye, an alkali, a reducing agent suitable for printing, a gum thickening agent, and a quaternary base compound of the general formula:



65 where  $R_1$ ,  $R_2$ ,  $R_3$  and  $R_4$  are the same or different alkyl or aralkyl groups, one at least of which is an alkyl group containing a hydroxy group, and where  $X$  represents  $-\text{OH}$  or an acid residue, and thereafter developing the print.

RONALD TONKIN.  
JAMES STEVENSON WILSON. 75